

Patented Aug. 19, 1952

2,607,486

Process for the flotation of iron oxide ore from siliceous gangue minerals, and the resulting product.

John W. Barr, Jr., Evanston, Ill., assignor to  
Armour and Company, Chicago, Ill., a corpora-  
tion of Illinois

# UNITED STATES PATENT OFFICE

2,607,486

## IRON OXIDE FLOTATION PROCESS

James A. Barr, Jr., Evanston, Ill., assignor to  
Armour and Company, Chicago, Ill., a corpora-  
tion of Illinois

No Drawing. Application August 30, 1946,  
Serial No. 694,170

3 Claims. (Cl. 209—166)

1

This invention relates to an iron oxide flotation process, and more particularly to the use of an improved collector agent in the flotation of iron oxide ore from siliceous gangue minerals.

In the flotation of iron oxide from siliceous gangue minerals, certain sulfonated or sulfated oils have been employed, including tall oil, and with varying degrees of success. Tall oil, which is obtained from the "black liquor" residue of pulp wood in the manufacture of paper is available commercially in large quantities, but the product has not been very successful as a collector material in the flotation of iron oxides.

I have discovered that when tall oil is fractionated to produce a fraction which is rich in linoleic acid and this fraction is then sulfated or sulfonated, an unusually effective collector is provided for use in the flotation of iron oxides. I have further discovered that the new advantages in yield and effectiveness as a collector are obtained by reason of the linoleic acid content of the product and that linoleic acid obtained from any source, when sulfated or sulfonated, becomes extremely efficient as a flotation collector for iron oxide ore.

An object of this invention is to provide a process for the flotation of iron oxide ore from siliceous gangue mineral in which sulfated or sulfonated linoleic acid derived from any source is employed as a collector. A further object is to provide a process in which a fraction of tall oil which is rich in linoleic acid, containing more than the natural concentration of linoleic acid in tall oil, is sulfated or sulfonated and employed as a collector in the flotation of iron oxide. Yet another object is to provide a process in which tall oil from which the abietic acid has been substantially removed, is sulfonated or sulfated and the resulting product employed as a flotation collector for iron oxide ore. Yet another object is to provide a process for the flotation of iron oxide ore from siliceous gangue minerals in which a sulfonated or sulfated fatty acid containing multiple double bonds is employed as a collector agent. Other specific objects and advantages will appear as the specification proceeds.

My new process, in one embodiment, comprises the use of a sulfated or sulfonated fatty acid containing multiple double bonds. In the flotation of iron oxide ore from siliceous gangue minerals, the mixture is passed through the usual flotation circuits and aerated to bring the oxide-carrying froth to the surface for removal. Linoleic acid, whether derived from tall oil or from

any other source, is effectively employed. The flotation operation is the same as that ordinarily employed except with respect to the particular flotation collector described, and it is believed, therefore, that a detailed description of the flotation steps as ordinarily practiced need not be set out in detail herein.

Because of the large quantities of tall oil available as a by-product of the paper industry and 10 because of certain desirable qualities of tall oil with respect to coating the surface of the iron oxide ore, I prefer to employ a sulfated or sulfonated tall oil fraction which is rich in linoleic acid. For example, tall oil may be fractionally 15 distilled to obtain separately various fractions, some of which contain no linoleic acid and others of which contain materials which are undesired for the flotation process. For example, the bulk 20 of the rosin or abietic acid may be removed in the distillation process, and the remainder of the product which is rich in linoleic acid may be employed successfully in the process. Further, the palmitic acid and some unsaponifiable matter obtained as a low boiling fraction may be 25 removed. The pitch, which is naturally obtained as a residue product in the fractional distillation, may also be eliminated. The remaining fraction is rich in linoleic acid, containing more 30 than twice the natural concentration of linoleic acid in the tall oil, and the product when sulfonated or sulfated, is unusually effective as a collector material in the flotation process.

In the fractional distillation of tall oil, a fraction 35 is readily obtained which contains oleic acid and linoleic acid, together with a little abietic acid. This fraction may be fractionally crystallized with a suitable solvent, such, as for example, acetone, and after the removal of the solid fraction there is obtained a product which 40 is extremely rich in linoleic acid. This product after sulfonation or sulfation is extremely efficient as a flotation collector for iron oxide ore in removing it from siliceous gangue minerals.

As specific examples, the following may be set 45 out:

The iron oxide mixed with siliceous gangue minerals, as recovered from the mine, was ground to the usual mesh fineness and pulped with water in the flotation circuit and in contact with a collector comprising a sulfonated tall oil fraction consisting principally of linoleic acid mixed with oleic acid. Air was introduced in the usual manner at the bottom of the flotation cell and 50 the froth formed carried the iron oxide ore to

which the sulfonated tall oil fraction was attached to the surface.

In a second example, the procedure was the same as that stated in the above example except that the collector agent consisted of sulfated tall oil from which abietic acid had been removed.

In a third example, the process was the same as described in example one above, but the collector was sulfonated linoleic acid.

As a standard of comparison for the above tests, I carried through a similar operation which was identical with example one except that sulfonated crude tall oil was employed as the collector. The yields obtained by the use of linoleic acid and of the fractions of tall oil rich in linoleic acid greatly exceeded the yields obtained by the use of sulfonated tall oil, demonstrating that the efficient recovery of iron oxide from the siliceous gangue minerals was due to the predominance of linoleic acid in the sulfonated or sulfated material.

I find that the effective material in the flotation step is the sulfonated or sulfated fatty acid containing multiple double bonds, and all fatty acids of this character respond as efficient flotation collectors with respect to iron oxide.

While in the foregoing description I have set forth certain embodiments of the invention as illustrative and in considerable detail, it will be

understood that such details may be varied widely by those skilled in the art without departing from the spirit of my invention.

I claim:

1. In a process for the separation of iron oxide from siliceous gangue minerals in a flotation operation, the steps of subjecting the ground minerals in water to the action of a collector selected from the group consisting of sulfonated and sulfated tall oil fractions having a content of linoleic acid greater than that occurring naturally in tall oil, and from which the bulk of the abietic acid has been removed.

2. In a process for the separation of iron oxide from siliceous gangue minerals in a flotation operation, the steps of subjecting the ground minerals in water to the action of a collector selected from the group consisting of sulfated and sulfonated tall oil fractions consisting predominantly of linoleic acid.

JAMES A. BARR, JR.

#### REFERENCES CITED

The following references are of record in the file of this patent:

#### UNITED STATES PATENTS

| Number    | Name  | Date           |
|-----------|-------|----------------|
| 2,385,054 | Booth | Sept. 18, 1945 |
| 2,414,714 | Booth | Jan. 21, 1947  |